

Oct. 15, 1968

K. J. RADIMER ET AL

3,406,108

REGENERATION OF SPENT AMMONIUM PERSULFATE ETCHING SOLUTIONS

Filed Oct. 1, 1965



INVENTOR.  
KENNETH J. RADIMER  
FRANK J. CAROPRESO  
BY *Frank J. Radimer*  
*Eugene J. Serrao*  
*Milton Zucker*

## 1

3,406,108

REGENERATION OF SPENT AMMONIUM  
PERSULFATE ETCHING SOLUTIONS

Kenneth J. Radimer, Little Falls, and Frank E. Caropreso, Hamilton, N.J., assignors to FMC Corporation, New York, N.Y., a corporation of Delaware  
Continuation-in-part of application Ser. No. 451,635, Apr. 28, 1965. This application Oct. 1, 1965, Ser. No. 495,374

23 Claims. (Cl. 204—82)

This invention relates to the recovery of unused persulfate values in spent etching solutions, and further, to the regeneration of spent ammonium persulfate etching solutions.

This application is a continuation-in-part of patent application Serial No. 451,635, filed Apr. 28, 1965, and now abandoned, in the names of Frank E. Caropreso, Kenneth J. Radimer and Bernard J. Hoga.

Solutions of peroxygen chemicals such as ammonium persulfate are commonly used to dissolve metals such as copper, cobalt, iron, nickel and zinc. This is desirable, for example, in place of ordinary machining in order to remove specified amounts of these metals from surfaces of fragile or peculiarly shaped objects. A more widespread application of this technique is the production of printed electrical circuits. In this application a resist or mask in the form of the desired circuit is placed over the surface of a copper film laminated to a base, and the partially masked copper film is treated with the etchant. The copper area not covered by the resist is dissolved, while the copper covered by the resist remains to form the desired circuit.

Ammonium persulfate solutions are desirable in such applications because they do not generate obnoxious fumes, are easy to work with, and are relatively non-corrosive to certain common materials of construction such as stainless steels. In use, the metal, e.g., copper is dissolved in the nonmasked areas by the persulfate solution until the dissolution rate is below commercially acceptable rates. The resulting spent etchant must be treated to remove the dissolved metal, e.g., copper before it is sewered.

One serious problem that has arisen in using this process is that substantial amounts of persulfate are discarded in the spent etchant. It has not been possible to recover or make use of these remaining persulfate values in the spent etchant on a commercial scale; the mere addition of fresh ammonium persulfate to a spent etching solution to restore the original persulfate concentration does not yield an acceptable etching solution because such solutions give inferior and erratic etching.

A second problem is that the treatment of spent persulfate solutions to remove metal values, e.g., copper, entails an additional process step which adds to the expense of disposing of these solutions. Copper must be removed from the persulfate solutions before they are sewered because of the toxicity of the copper values.

One method of eliminating the expense of disposing of spent etching solutions is set forth in our parent application Serial No. 451,635 wherein said solutions are cooled to a temperature sufficient to crystallize copper sulfate values and ammonium sulfate values from the solution without crystallizing substantial amounts of ammonium persulfate; the crystallized solids can be separated from the remaining solutions which then can be used for etching. This parent application also provides for adding additional ammonium persulfate values to the reactivated solution when desired. This process is helpful in solving the waste disposal problem and in utilizing residual persulfate values in the spent etchant, but it does not set forth a technique for regenerating persulfate from the remaining values in the spent solution.

## 2

As a result there has been a need for a method of treating spent persulfate etching solutions on a commercially acceptable basis to recover the residual persulfate values, to regenerate additional persulfate values and to eliminate the disposal problems associated with spent persulfate solutions.

It is an object of the present invention to treat spent ammonium persulfate etching solutions to satisfy these needs.

It is a further object of the present invention to obviate these difficulties by treating spent persulfate etching solutions to remove the metal values, e.g., copper, present in the etching solution and to regenerate the persulfate values in said etching solution so as to obtain etchants yielding consistent, commercially acceptable etching rates.

We have found that a spent aqueous ammonium persulfate etching solution which has been used to dissolve a metal such as copper, cobalt, iron, nickel and zinc, and which contains the corresponding metal sulfate, ammonium sulfate and residual ammonium persulfate values can be regenerated by treating said solution to remove a substantially persulfate-free mixture containing ammonium sulfate and the corresponding metal sulfate, using the persulfate-free mixture as the catholyte of an electrolytic cell, using the remainder of said spent solution containing sulfate values and residual persulfate values as the anolyte of said electrolytic cell, the cathode and anode sections of the electrolytic cell being contained in a manner (preferably separated by a diaphragm) which permits at least hydrogen ions to pass freely between the anolyte and catholyte but which prevents any substantial amounts of persulfate in the anolyte from mixing with the catholyte, passing an electric current through said catholyte and anolyte by means of a cathode in said catholyte and an anode in said anolyte, plating out said metal at said cathode, producing persulfate values at said anode, obtaining a catholyte substantially reduced in metal content, and recovering an anolyte solution having an increased persulfate content and suitable as a regenerated etching solution.

It has further been found that regeneration of the persulfate values at the anode is facilitated by carrying out the regeneration in the presence of urea or ammonium thiocyanate ( $\text{NH}_4\text{CNS}$ ) in the anolyte.

In the following detailed description of the invention, the process will be described with reference to regenerating ammonium persulfate solutions which have been used to etch copper. However, it should be understood that copper is only illustrative of one embodiment and that substantially the same effect can be obtained with cobalt, iron, nickel or zinc.

In carrying out the present invention a fresh aqueous 0.75 to 1.25 molar (M) ammonium persulfate etching solution (containing from about 171 g. to 285 g. of ammonium persulfate per liter of water) can be heated to temperatures of from about 35° to 46° C. and used to etch unmasked portions of copper. The etching can take place either by conventional immersion etching or spray etching. In the immersion etching process the masked copper workpiece is immersed in the solution for the amount of time required to etch the exposed copper surface. In the spray etching technique the persulfate solution is discharged from a spray nozzle under pressure and the spray impinges on the masked copper workpiece.

In practice, the spray etching technique is preferred because it permits shorter etching times and results in a better quality etch. This is due in large measure to the constant replacement of the copper-rich layer of etchant in immediate contact with the workpiece with fresh etchant.

Etching can be continued until the solution has been

depleted of persulfate values to a concentration of about 0.4 to 0.6 M ammonium persulfate. At this point, the solution is capable of further etching, but the etch rate and quality of etch diminishes and such solutions are normally discarded as "spent" solutions.

In accordance with a preferred embodiment, this "spent" solution is passed to a crystallizer, preferably a vacuum crystallizer, which is maintained at a temperature of 0° to 20° C., whereupon copper sulfate and ammonium sulfate crystallize leaving substantially all the persulfate values in the remaining mother liquor. The exact temperature of cooling is not critical but it should be sufficiently low to crystallize substantial amounts of copper sulfate and ammonium sulfate, normally in the form of a hydrated double salt, but not ammonium persulfate values. A temperature of about 0° to 10° C. is optimum. In many cases vacuum crystallizers are desired in order to remove some of the water in the remaining solution.

The resulting crystals are separated from the solution by filtering or by centrifugal separators. During the separation care must be taken to remove adhered mother liquor from the precipitate in order to prevent loss of ammonium persulfate values. The precipitated crystals are then dissolved in water and passed into the cathode section of an electrolytic cell for use as a catholyte. It is critical that the catholyte be free of any substantial amounts of persulfate since the presence of persulfate interferes with the proper functioning of the electrolytic cell.

The mother liquor from the crystallization step which contains the remaining copper, ammonium and "sulfate values" as well as the residual persulfate values, is passed into the anode section of the above electrolytic cell and used as an anolyte. The term "sulfate values" as used in the specification and claims refers to both sulfate and bisulfate water-soluble compounds.

The anolyte and catholyte solutions must be contained in a manner to prevent any substantial amounts of persulfate values in the anolyte from mixing with the catholyte, but without preventing the flow of an electric current between these solutions. Separation of the solutions by differences in specific gravity is workable but best results are achieved by placing a diaphragm between the two solutions. The diaphragm permits the flow of an electric current between the anolyte and catholyte, but prevents substantial amounts of persulfate in the anolyte from diffusing into the catholyte. The flow of current between the anolyte and catholyte takes place by passing certain ions, principally hydrogen ions, through the diaphragm and is a necessary part of the electric circuit of the cell. The diaphragm in the electrolytic cell can be any porous membrane such as a porous porcelain sheet, asbestos membrane, plastic membranes, etc.

An electrode then is immersed in each catholyte and anolyte solution. These electrodes can be any material which can conduct an electric current and which does not react with the solutions of the cell during the electrolysis. Generally, noble metals such as platinum or gold are preferred as anodes, and copper is preferred as the cathode, since copper plates out on the cathode in the ensuing reaction. An electric potential is placed across the electrodes (the anode and cathode) by means of a battery, rectifier or other source of direct current to complete the electrolytic cell.

The electric potential which is applied across the electrodes must be sufficient to cause a positive electrical current to flow outside the cell from cathode to anode to plate out copper at the cathode and convert sulfate values to persulfate at the anode. Normally an EMF of at least about 2.5 volts has been found operable with from about 5 to 7 volts being preferred. The electrolytic regeneration is conducted at a temperature of from about 2° to 30° C. with temperatures from about 5° to 20° C. being pre-

ferred. The EMF and current which are used in operating the cell are not critical and may be varied depending upon the rate of regeneration which is desired.

The regeneration has been found to proceed with greater efficiency in the conversion of sulfate values to persulfate when urea or ammonium thiocyanate



is present in the anolyte in concentrations of up to about 0.2%. The presence of urea or  $\text{NH}_4\text{CNS}$  in amounts of about 0.005% has been found most effective in increasing anode efficiency for the production of persulfate from sulfate by 50 to 100%. The presence of urea or  $\text{NH}_4\text{CNS}$  in the catholyte does not interfere in any manner with the regeneration or operation of the electrolytic cell.

In general, a cathode having a large surface area is used to facilitate copper deposition while the anode can have a much smaller surface area. Thus, in typical operations, current densities from 25 to 30 amps per square foot at the cathode and 1100 amps/sq. ft. at the anode have been used with good effect.

The desired half-reactions for each of the half cells are as follows:

At the cathode—



At the anode—



The desired overall reaction of the electrolytic cell is



In the above described regeneration, current efficiencies for production of persulfate at the anode are improved by the presence of high concentrations of sulfate values in the anolyte. Normally, the cell diaphragm does not permit ready transfer of sulfate values from catholyte to anolyte to replace sulfate values which are converted to persulfate. To provide enough sulfate values to the anolyte for the production of high concentrations of persulfate it is desirable to introduce additional sulfate values into the anolyte in order to augment existing sulfate values. This can be done by introducing these additional sulfate values directly into the spent etchant before copper ammonium sulfate is crystallized from it. Such added sulfate values must be capable of passing into the mother liquor during the crystallization step.

Ammonium bisulfate is preferred as a source of supplementary sulfate values because it does not introduce foreign ions into the anolyte solution. Other soluble compounds which increase the anolyte's sulfate concentration can also be used providing that they do not interfere with the electrolytic regeneration or with the subsequent etching. Sulfate values might be increased by introducing materials such as ammonium sulfate, sodium sulfate, or sulfuric acid.

The supplementary sulfate values are preferably introduced into the spent etchant before crystallization of copper and ammonium sulfate from it, as set forth above, in order to increase the extent of crystallization of copper values from the aqueous solution; this solution after being electrolyzed has therefore a lower copper concentration which leads to better etching. Alternatively, the added sulfate values can be introduced directly into the mother liquor subsequent to crystallization. In either case the sulfate values in the mother liquor, which pass into the anolyte, are increased.

In general, one continues electrolysis at least until copper is completely removed from the catholyte. This removal of copper is accompanied by a transfer of hydrogen ions through the membrane from anolyte to catholyte, hydrogen ions having the highest mobility of any of the dissolved species, and the catholyte thus becomes substantially a solution of ammonium bisulfate. Electrolysis of the catholyte beyond this point does not change

its chemical composition greatly since any hydrogen ions which are reduced at the cathode are replaced by hydrogen ions diffusing through the membrane.

The electrolysis can be conducted batchwise or continuously. In a continuous operation electrolytic cells should be used in which the electrolytes are introduced at one end of the cell and flow along the membranes until they are removed from the cell at the opposite end. During this flow reduction of the copper concentration in the catholyte and an increase in the persulfate concentration in the anolyte occur. The solutions can be introduced into other such cells in cascade if desired.

When regeneration has been completed the persulfate-rich anolyte is passed to the etching machine and the exit catholyte is passed to an evaporator. In the course of the electrolysis the persulfate concentration of the anolyte can be raised to any extent desired up to about 0.8 to 1.0 M; such solutions have been found to be acceptable etchants. In the evaporator, water is stripped from the exit catholyte. The resulting concentrated catholyte contains sulfate values, principally as ammonium bisulfate, and is useful for supplying supplementary sulfate values required in subsequent anolytes as described above. In any event the final catholyte contains virtually no copper and therefore can be seweried if the ammonium bisulfate values are not desired.

In general it is preferred to continue electrolysis until all the copper has been completely plated at the cathode and to operate the cell with anolyte concentrations such that an amount of persulfate, equivalent to the amount of plated copper, is produced in the same period. It has occasionally been found that it is desirable to continue electrolysis somewhat beyond the point at which all of the copper at the catholyte has been plated out in order to produce the desired persulfate concentration in the anolyte.

In the above description of the invention a crystallization procedure was used in order to prepare a persulfate-free catholyte. As an alternate to crystallization, a portion of the etchant intended for use as catholyte may be treated to decompose persulfate values. This may be done for example by merely heating that portion of the etchant to a temperature between about 50° C. and 100° C. at which temperature the persulfate decomposes. Alternately, the residual persulfate in this portion of the etchant may be destroyed by reacting it with a chemical reducing agent such as sulfur dioxide. The resulting etching solution, free of residual persulfate, can then be used as the catholyte. Untreated spent etchant, which still contains residual persulfate, may be used as the anolyte. The electrolytic regeneration is carried out using these solutions as catholyte and anolyte, respectively, in the same manner as set forth previously.

In the above description of the invention the desirability of adding supplementary sulfate values to the anolyte to improve anode efficiency in producing persulfate has been described. These sulfate values, preferably in the form of ammonium bisulfate can be supplied from any available source including the exit catholyte, once cyclic regeneration has commenced. However, to start up the process such supplementary sulfate values can be obtained in the form of copper ammonium sulfate crystals. These can be obtained by cooling some spent etchant to 0° to 20° C. to precipitate these crystals, and adding the crystals to the anode chamber during electrolysis.

An alternate method is to manufacture ammonium bisulfate for use in start up. One method is to cool spent etchant to obtain crystals, redissolve these crystals in water for use as a catholyte, and use the mother liquor as the anolyte. Upon electrolysis of this cell, ammonium bisulfate is formed in the catholyte which can be used as a source of supplementary sulfate values.

One embodiment of the invention that is contemplated to enable an ammonium persulfate solution to be used indefinitely for etching is carried out by continuously re-

moving a portion of the etching solution, continuously adding concentrated exit catholyte thereto, cooling the resulting solution to precipitate sulfate insolubles and continuously removing sulfate insolubles from the supernatant solution. The sulfate insolubles (free of persulfate) are dissolved in water continuously and this solution continuously fed to the cathode compartment of an operating electrolytic cell; the remaining supernatant solution in similar fashion is fed continuously in the anode compartment of the electrolytic cell. The resulting electrolytic regeneration increases the persulfate values in the anode compartment of the electrolytic cell while converting copper ions to copper metal in the cathode compartment. The regenerated anolyte, enriched in persulfate values, is removed from the cell and recycled back to the main body of etching solution continuously. The exit catholyte, substantially free of copper, is passed continuously into an evaporator to remove some of its water. The resulting concentrated exit catholyte is removed and continuously added to the stream of spent etchant prior to the cooling and crystallizing step as described above.

The resulting etching solution in such a process thus can be used continuously with this cyclic crystallization and regeneration procedure unless or until foreign impurities which may be introduced inadvertently or build up in the solution to a point where the quality of etch is affected. Such a process obviates the need for replacing etching solution and for disposing of the spent solutions or other waste materials.

In general the quality of etch obtained by using regenerated persulfate solution is about the same as that obtained with fresh ammonium persulfate solution. Thus the electrolytic regeneration technique described above does not entail any reduction in the high quality of etch obtained when using ammonium persulfate etchants.

The present invention will now be described by reference to the drawing which is a diagrammatical flow sheet of the process.

In the drawing an ammonium persulfate etching solution is heated in an etching machine 2 and used to etch photo-resisted, copper laminated printed circuit panels until the rate and quality of etch are no longer commercially acceptable. The spent solution is then withdrawn from the etching machine 2 and transferred to a vacuum crystallizer 4 in which the contents are cooled to a temperature of 0° to 10° C. In the vacuum crystallizer 4 some water is vaporized during cooling and sent to condenser 24; during cooling crystals of copper ammonium sulfate are precipitated. These crystals, which contain substantially no ammonium persulfate, are separated from the mother liquor in centrifuge 6. The mother liquor which contains copper sulfate, ammonium sulfate, ammonium bisulfate and residual ammonium persulfate is then discharged into the anode compartment 8 of an electrolytic diaphragm cell 10 for use as the anolyte. The copper ammonium sulfate crystals are dissolved in water obtained from water storage tank 26 and discharged into the cathode compartment 12 of the diaphragm cell 10. The diaphragm cell 10 is made up of an anode compartment 8 and a cathode compartment 12 separated by a diaphragm 14 through which hydrogen ions can pass, but which prevents any substantial diffusion of other ions from one side of the diaphragm to the other. The diaphragm must prevent substantial amounts of persulfate ions from diffusing from the anode to the cathode compartment. Where desired, the free surface of the catholyte in the cathode compartment 12 can be maintained slightly higher than that of the anolyte in the anode compartment 8 to diminish such diffusion. The anolyte and catholyte are electrolyzed by passing a direct current through the anode 16 immersed in the anolyte and through the cathode 18 immersed in the catholyte. The direct current is supplied by battery 20 or other equivalent source of direct current. Within the cell electrical current is carried between the

anode and cathode by the ions which diffuse through the diaphragm.

During electrolysis, copper ions in the catholyte are converted to metallic copper and are plated out on the cathode 18. Sulfate values in the anolyte simultaneously are converted at the anode 16 into persulfate ions. The diaphragm cell 10 is properly operating when the quantity of copper plated out at the cathode 18 is approximately equivalent chemically to the amount of persulfate produced in the anolyte. Electrolysis is continued until all the copper from the catholyte has been plated out on cathode 18 and the desired concentration of persulfate has been reached in the anolyte compartment 8. The exit anolyte, rich in persulfate, is recycled back to the etching machine 2 for further etching. The exit catholyte from cathode compartment 12, which contains virtually no copper but which is rich in ammonium bisulfate, is transferred to evaporator 22 where a substantial amount of its water is removed. The water vapor is condensed in condenser 24 and passed to a water storage tank 26. The ammonium bisulfate concentrate from evaporator 22 may then be passed to the vacuum crystallizer 4 or directly to the anode compartment 8 of the diaphragm cell 10. In either case, the ammonium bisulfate flows to the anolyte as supplementary sulfate values; however, it is preferred to pass the concentrate into the vacuum crystallizer 4 along with spent etchant in order to increase the efficiency of copper removal from the etchant during crystallization in vacuum crystallizer 4.

In the above illustrated process no chemicals need be added to the system after it has been put into operation, except for small operating losses, e.g., such as loss of chemicals in solutions adhering to etched printed circuits. Further, no by-products or waste materials are produced. The net effect of this system's operation is solely the movement of copper metal from the printed circuit board onto the copper cathode. All other chemicals remain in balance, and the applied electrical current merely reconverts sulfate values to persulfate values. The system defined in the drawing is exemplified in Example 1 wherein each unit operation is carried out in a batchwise manner before being passed on to the next unit operation.

In operating the above system properly so that the copper plated at the cathode is equivalent to the quantity of persulfate produced at the anode, it is sometimes necessary to continue electrolysis beyond the point at which all of the copper has been deposited from the catholyte. This can be minimized by adjusting the solute concentrations in the electrolytes.

In the embodiment of the above illustrated process which is described in Example 1 the process has been carried out by etching batchwise with a quantity of etchant until all of the etchant is spent and then treating the entire etchant in each of the unit operations in sequence until the etchant is finally regenerated. However, it is within the contemplated scope of this invention to withdraw continuously only a portion of the etching solution in a constant stream and to regenerate this stream of withdrawn etchant constantly by continuous treatment in each unit, namely, the vacuum crystallizer, centrifuge and diaphragm cell. The regenerated stream of withdrawn etchant is then recycled continually to the etching machine.

Operation in such a completely continuous manner has the advantage that each of the units, and most importantly the etching machine, would be in continuous operation and the concentration of solutes in the etchant could be maintained constant. This would result in highly desirable constant etching rates and reduce the amount of maintenance required to keep the etching precise and within commercial tolerances. This system would also lend itself to automation most readily since it is a balanced system in which the chemical solutions would be recycled throughout the units without varying in solute concentrations at any point in the system.

The following examples are given to illustrate the present invention and are not deemed to be limiting thereof.

#### EXAMPLE 1

5 A process for regenerating an etching solution was carried out as follows. An etchant solution was prepared containing 1.1 moles of ammonia persulfate per liter and 5 p.p.m. of dissolved mercury as  $HgCl_2$  which is the etching catalyst. This was used to etch photo-resisted, 10 single-sided printed circuit test panels, the copper foil of which weighed 1 oz. per sq. ft. The etching was conducted by immersing the test panels in the air-agitated etchant at a temperature of 35-39° C. Etching rates and 15 the quality of etch were determined frequently during the run and were found to be satisfactory. When the etch rate dropped below about 0.2 mil of copper per minute, the etchant was considered to be spent. At this point one liter of it contained:

|                  | Mole |
|------------------|------|
| 20 Persulfate    | .61  |
| Dissolved copper | .45  |
| Sulfate values   | .94  |

25 To one liter of this spent etchant .55 mole of  $NH_4HSO_4$  was added. The resulting solution was cooled to 2-5° C. by vaporization of some water from it at a pressure of about 5 mm. of mercury. Blue crystals containing copper and ammonium sulfates were precipitated from the solution, they were separated from their mother liquor 30 using a Büchner funnel and were identified as



35 Analysis indicated that about .26 mole had formed. The crystals were dissolved in water. Both the solution of the crystals and the mother liquor were analyzed with the following results:

|                  | Mother liquor, mole | Crystal solution, mole |
|------------------|---------------------|------------------------|
| 40 Persulfate    | .59                 | .02                    |
| Dissolved copper | .21                 | .26                    |
| Sulfate values   | .98                 | .52                    |

45 The mother liquor was added to the anode compartment of a diaphragm cell; urea was added to give a .02% solution. The crystal solution was passed into the cathode compartment of the same diaphragm cell. A platinum wire was suspended in the anode compartment to serve as an anode, while copper tubing was used as a cathode in contact with the crystal solution in the cathode compartment of the cell. The anode and cathode were connected to a rectifier and electrolysis was conducted for about 11 hours using a current of about 3 amperes. The current density was about 1100 amps./sq. ft. at the anode and about 30 amps./sq. ft. at the cathode. 55 The temperature of the anolyte and catholyte was about 20-25° C. and 18-20° C., respectively, during electrolysis. After electrolysis the anolyte and catholyte were analyzed with the following results:

|                  | Anolyte, mole | Catholyte, mole |
|------------------|---------------|-----------------|
| 60 Persulfate    | .87           | None            |
| Dissolved copper | .21           | Trace           |
| Sulfate values   | .42           | .56             |

65 After the electrolysis was completed, water was evaporated from the exit catholyte. Enough water was evaporated at this point and in the vacuum crystallization to provide at least as much water as was used in preparation of the catholyte. The anolyte was used for etching another series of printed circuit test panels, after which 70 it was analyzed with the following results:

|                  | Mole |
|------------------|------|
| 75 Persulfate    | .61  |
| Dissolved copper | .47  |
| Sulfate value    | .95  |

Quantities of materials noted above in the example have been corrected for amounts removed on analytical samples.

In the above example the amounts of ingredients found in the reused etchant and in the exit catholyte were considered to correspond closely enough to those in the spent etchant and bisulfate additive used in the previous regeneration to assure that any number of additional crystallization, separation and electrolysis cycles could be run using substantially the same amounts of materials in each step and obtaining substantially the same results.

### EXAMPLE 2

A series of runs was made, in which photo-resisted, single-sided, 1 oz./sq. ft., copper laminated printed circuit test panels were etched. In these runs 500 ml. portions of a fresh aqueous etching solution, each having an ammonium persulfate concentration of about 1 M and 5 p.p.m. of  $HgCl_2$  (which is used as the etching catalyst), were used to etch the abovementioned circuit test panels until the solutions were about 50% depleted of their ammonium persulfate. The etching was conducted by immersing the test panels in the air-agitated etchant maintained at a temperature of 38-39° C. The average etching rates were on the order of from about 0.25 to about 0.30 mils of copper per minute and the quality of etch obtained was good. In general, an etch rate of about 0.2 mil of copper per minute is considered acceptable for commercial use.

The spent etching solutions were cooled to a tempera-

5 was suspended in the cup and served as the anode while a copper tubing 0.25 in. in diameter was wrapped in a helix around the porous cup and served as the cathode. Water was passed through the copper tubing for better temperature control. The anolyte was continually 10 agitated by means of a Teflon-coated magnetic stirring bar placed in the base of the porcelain cup. The anode and cathode were connected to a rectifier which supplied direct current. The electrolytic cell was operated by adjusting the voltage passing through the cell to give the desired current. Each of the solutions in Runs 1-4 was subjected to electrolysis for 60 minutes.

15 The ammonium persulfate contents of the anolyte solutions both prior to and subsequent to regeneration were determined by addition of a known excess of standard ferrous ammonium sulfate and back titration with standard potassium permanganate. The compositions of the anolyte and catholyte prior to electrolysis are given in Table I along with the final persulfate contents of the anolytes. The conditions under which electrolysis 20 was carried out are also set forth in Table I. In Run 3, sulfuric acid was added to the anolyte to supply additional sulfate values for conversion to persulfate. In Run 4, 0.02% by weight of urea was added to the anolyte and catholyte to increase the anode efficiency for production of persulfate.

25 The regenerated anolyte solution from Run 4 was used as a regenerated etchant to etch test panels identical to those etched by the initial etchant. The rate of etch was 30 found to be substantially above 0.2 mil of copper per minute and the quality of etch was good.

TABLE I

| Run | Initial Electrolyte Composition                                                                                 |                                                                            | Final<br>( $NH_4$ ) <sub>2</sub> S <sub>2</sub> O <sub>8</sub><br>Content of<br>Anolyte | Amps | Volt       | Current Density,<br>Amps/Ft. <sup>2</sup> |         | Temperatures, °C. |         | Electrode<br>Efficiency, Percent |         |
|-----|-----------------------------------------------------------------------------------------------------------------|----------------------------------------------------------------------------|-----------------------------------------------------------------------------------------|------|------------|-------------------------------------------|---------|-------------------|---------|----------------------------------|---------|
|     | Anolyte                                                                                                         | Catholyte                                                                  |                                                                                         |      |            | Anode                                     | Cathode | Anolyte           | Cathode | Anode                            | Cathode |
| 1   | { 0.48 M ( $NH_4$ ) <sub>2</sub> S <sub>2</sub> O <sub>8</sub><br>0.5 M CuSO <sub>4</sub>                       | { 0.5 M ( $NH_4$ ) <sub>2</sub> SO <sub>4</sub><br>0.5 M CuSO <sub>4</sub> | 0.61M                                                                                   | 3    | 6.2 to 8.2 | 1,150                                     | 37      | 25                | 18      | 23                               | 96.0    |
| 2   | { 0.46 M ( $NH_4$ ) <sub>2</sub> S <sub>2</sub> O <sub>8</sub><br>0.5 M ( $NH_4$ ) <sub>2</sub> SO <sub>4</sub> | { 0.5 M CuSO <sub>4</sub><br>0.5 M CuSO <sub>4</sub>                       | 0.58M                                                                                   | 3    | 5 to 5.8   | 1,150                                     | 25      | 26                | 22.5    | 22                               | 84.6    |
| 3   | { 0.5 M ( $NH_4$ ) <sub>2</sub> S <sub>2</sub> O <sub>8</sub><br>0.4 M CuSO <sub>4</sub>                        | { 0.5 M ( $NH_4$ ) <sub>2</sub> SO <sub>4</sub><br>0.5 M CuSO <sub>4</sub> | 0.71M                                                                                   | 3    | 5 to 5.4   | 1,150                                     | 37      | 23                | 18      | -----                            | -----   |
| 4   | { 0.51 M ( $NH_4$ ) <sub>2</sub> S <sub>2</sub> O <sub>8</sub><br>0.5 M CuSO <sub>4</sub>                       | { 0.5 M ( $NH_4$ ) <sub>2</sub> SO <sub>4</sub><br>0.5 M CuSO <sub>4</sub> | 0.74M                                                                                   | 3    | 5.5 to 7.0 | 1,150                                     | 25      | 27                | 22      | 40                               | 91.6    |
|     | { 0.02% urea                                                                                                    | { 0.02% urea                                                               |                                                                                         |      |            |                                           |         |                   |         |                                  |         |

ture of about 2-3° C. using a vacuum type crystallizer operating at a vacuum of about 5 mm. of mercury. Blue crystals containing copper sulfate and ammonium sulfate values precipitated from the solutions; these crystals were identified as  $CuSO_4(NH_4)_2SO_4 \cdot 6H_2O$ . The crystals were filtered from the mother liquor and sufficient water was added to the crystals to make a solution of 0.5 M copper sulfate and 0.5 M ammonium sulfate. These solutions were used as the catholytes in subsequent electrolytic regenerations. Water was added to the mother liquor to replace that removed during the vacuum crystallization until solutions containing about 0.5 M ammonium persulfate were obtained; these were used as the anolytes in the electrolytic cell during the regeneration process.

The electrolytic cell comprises a porous porcelain cup standing in a larger glass beaker. The porous cup contained the anolyte and the area between the cup and the glass beaker contained the catholyte. The porous cup served as the diaphragm to retard diffusion of persulfate from the anolyte (contained in the cup) to the catholyte (contained in an annular space between the cup and the glass beaker). A platinum wire 0.04 in. in diameter

### EXAMPLE 3

55 A series of runs were made in substantially the same manner as set forth in Example 2, Run 1, except that in place of copper the spent etchant contained either cobalt, iron, nickel or zinc dissolved in the etchant. The spent etchant containing the ingredients and concentration level set forth in Table II, were cooled to a temperature given in Table II using a vacuum type crystallizer. Crystals were precipitated having the values set forth in Table II for each of the solutions. The crystals were filtered from the mother liquors and sufficient water was 60 added to these crystals to dissolve them. The resulting solutions were then used as the catholytes in subsequent electrolytic regenerations. The mother liquors which remained after vacuum crystallization were used as the respective anolytes in the above electrolytic regenerations. After operation of the electrolytic cells as set forth in Example 2, Run 1, the anolytes were analyzed to determine if there was an increase in persulfate concentration, while the cathodic chamber was observed to determine if the etched metal plated out on the cathode. The results 70 are given in Table II.

TABLE II

| Run    | Metal Etched | Spent Etchant Composition<br>(Molar Concentration) |                                                 |                         | Crystallizing<br>Temperature | Crystallized Values                   | Electrolyzed Solutions  |                                               |
|--------|--------------|----------------------------------------------------|-------------------------------------------------|-------------------------|------------------------------|---------------------------------------|-------------------------|-----------------------------------------------|
|        |              | NIH <sub>2</sub> S <sub>2</sub> O <sub>8</sub>     | (NH <sub>4</sub> ) <sub>2</sub> SO <sub>4</sub> | Metal Sulfate           |                              |                                       | Cathode                 | Anode                                         |
| 1..... | Cobalt.....  | 0.5                                                | 0.5                                             | 0.5 Cobalt sulfate..... | 0 to 2° C.....               | Cobalt sulfate, ammonium sulfate..... | Cobalt metal deposited. | Persulfate values increased in concentration. |
| 2..... | Iron.....    | 0.5                                                | 0.5                                             | 0.5 Iron sulfate.....   | -8° C.....                   | Iron sulfate, ammonium sulfate.....   | Iron metal deposited.   | Do.                                           |
| 3..... | Nickel.....  | 0.2                                                | 0.2                                             | 0.2 nickel sulfate..... | 0 to 2° C.....               | Nickel sulfate, ammonium sulfate..... | Nickel metal deposited. | Do.                                           |
| 4..... | Zinc.....    | 0.5                                                | 0.4                                             | 0.4 Zinc sulfate.....   | 0 to 2° C.....               | Zinc sulfate, ammonium sulfate.....   | Zinc metal deposited.   | Do.                                           |

Pursuant to the requirements of the patent statutes, the principle of this invention has been explained and exemplified in a manner so that it can be readily practiced by those skilled in the art, such exemplification including what is considered to represent the best embodiment of the invention. However, it should be clearly understood that, within the scope of the appended claims, the invention may be practiced by those skilled in the art, and having the benefit of this disclosure otherwise than as specifically described and exemplified herein.

What is claimed is:

1. A process for regenerating an ammonium persulfate etching solution which contains a dissolved metal selected from the group consisting of copper, cobalt, iron, nickel and zinc which comprises separating from said solution a persulfate-free mixture containing ammonium sulfate values and metal sulfate values corresponding to said dissolved metal and leaving a remaining solution containing sulfate values, adding said persulfate-free mixture into the cathode section of an electrolytic cell for use as a catholyte, adding said remaining solution containing sulfate values into the anode section of said electrolytic cell for use as an anolyte, said cathode and anode sections of said electrolytic cell being contained in a manner to prevent substantial amounts of persulfate values present in the anolyte from mixing with the catholyte, but permitting the free passage of at least hydrogen ions between said anolyte and said catholyte, passing an electric current through said catholyte and anolyte by means of a cathodic electrode contacting said catholyte and an anodic electrode contacting said anolyte, converting sulfate ions to persulfate ions at said anodic electrode, converting the dissolved metal ions to the corresponding metal at said cathodic electrode, and recovering an anolyte solution having an increased persulfate content.

2. The process of claim 1 wherein the dissolved metal is copper.

3. The process of claim 1 wherein the dissolved metal is zinc.

4. The process of claim 1 wherein the dissolved metal is iron.

5. The process of claim 1 wherein urea in amounts of from about 0.005% to 0.20% is added to said anolyte.

6. The process of claim 1 wherein ammonium thiocyanate in amounts of from about 0.005% to 0.20% is added to said anolyte.

7. The process of claim 1 wherein said electrolytic cell contains a diaphragm separating said anolyte and catholyte solutions.

8. A process for regenerating an ammonium persulfate etching solution which contains a dissolved metal selected from the group consisting of copper, cobalt, iron, nickel and zinc which comprises cooling said solution to crystallize metal sulfate values corresponding to said dissolved metal and ammonium sulfate values from said solution without crystallizing substantial amounts of ammonium persulfate, separating the crystallized solids from the remaining mother liquor, adding said crystallized solids to an aqueous liquor to make up a substantially persulfate-free mixture, adding said persulfate-free mixture into the cathode section of an electrolytic cell for use as a catholyte, adding the remaining mother liquor containing sulfate values into the anode section of the electrolytic cell

for use as the anolyte, said cathode and anode sections of said electrolytic cell being contained in a manner to prevent substantial amounts of persulfate values present in said anolyte from mixing with said catholyte but permitting the free passage of at least hydrogen ions between said anolyte and said catholyte, passing an electric current through said catholyte and said anolyte by means of a cathodic electrode contacting said catholyte and an anodic electrode contacting said anolyte, converting the dissolved metal ions to the corresponding metal at said cathodic electrode, converting sulfate ions to persulfate ions at said anodic electrode and recovering an anolyte solution having an increased persulfate content.

9. Process of claim 8 wherein the dissolved metal is copper.

10. Process of claim 8 wherein the dissolved metal is zinc.

11. Process of claim 8 wherein the dissolved metal is iron.

12. Process of claim 8 wherein said cooling is carried out at temperatures of from about 0° to 20° C.

13. Process of claim 8 wherein said cooling is carried out at temperatures of from about 0° to 10° C.

14. Process of claim 8 wherein said electrolytic cell contains a diaphragm separating said anolyte and catholyte solutions.

15. Process of claim 8 wherein urea in amounts of from about 0.005% to 0.20% are added to said anolyte.

16. Process of claim 8 wherein ammonium thiocyanate in amounts of from about 0.005% to 0.20% are added to said anolyte.

17. A process for regenerating an ammonium persulfate etching solution which contains dissolved copper which comprises mixing said etching solution with an aqueous ammonium bisulfate solution, cooling the resulting solution to crystallize copper sulfate and ammonium sulfate values from said resulting solution without crystallizing substantial amounts of ammonium persulfate, separating the crystallized solids from the remaining mother liquor, adding said crystallized solids to an aqueous liquor to make up a substantially persulfate-free mixture, adding said persulfate-free mixture into the cathode section of an electrolytic cell for use as the catholyte, adding the remaining mother liquor containing sulfate values into the anode section of the electrolytic cell for use as the anolyte, said cathode and anode sections of said electrolytic cell being contained in a manner to prevent substantial amounts of persulfate values present in said anolyte from mixing with said catholyte, but permitting the free passage of at least hydrogen ions between said anolyte and said catholyte,

passing an electric current through said catholyte and said anolyte by means of a cathodic electrode contacting said catholyte and an anodic electrode contacting said anolyte, converting copper ions to metallic copper at said cathodic electrode and forming ammonium bisulfate in said catholyte, converting sulfate ions to persulfate ions at said anodic electrode, passing the electrolyzed catholyte into an evaporator to remove water therefrom, recovering a concentrated ammonium bisulfate solution from said evaporator, and recovering an anolyte solution having an increased persulfate content and suitable as an ammonium persulfate etching solution.

18. Process of claim 17 wherein said electrolytic cell

contains a diaphragm separating said anolyte and catholyte solutions.

19. A process for regenerating an ammonium persulfate etching solution which contains dissolved copper which comprises cooling a first portion of said solution to obtain a first crystal precipitate containing copper sulfate values and ammonium sulfate values substantially free of ammonium persulfate, separating said first crystal precipitate from the remaining first mother liquor, adding said first crystal precipitate to an aqueous liquor to make up a substantially persulfate-free first mixture, adding said persulfate-free first mixture into the cathode section of an electrolytic cell for use as a catholyte, adding said first mother liquor containing sulfate values into the anode section of said electrolytic cell for use as the anolyte, said cathode and anode sections of said electrolytic cell being contained in a manner to prevent substantial amounts of persulfate values present in said anolyte from mixing with said catholyte but permitting the free passage of at least hydrogen ions between said anolyte and said catholyte, passing an electric current through said catholyte and said anolyte by means of a cathodic electrode contacting said catholyte and an anodic electrode contacting said anolyte, converting copper ions to metallic copper at said cathodic electrode and forming ammonium bisulfate in said catholyte, converting sulfate ions to persulfate ions at said anodic electrode, recovering a first anolyte solution having an increased persulfate content, recovering a first catholyte solution containing ammonium bisulfate and having a decreased copper content, recycling said first anolyte solution to said ammonium persulfate etching solution, dissolving additional copper with said ammonium persulfate etching solution, withdrawing a second portion of said solution and cooling said second portion of said solution to obtain a second crystal precipitate containing copper sulfate values and ammonium sulfate values substantially free of ammonium persulfate, separating said second crystal precipitate from the remaining second mother liquor, adding said second crystal precipitate to an aqueous liquor to make a substantially persulfate-free second mixture, adding said persulfate-free second mixture to said cathode section of an electrolytic cell for use as the catholyte, pass-

ing said second mother liquor containing sulfate values and said first catholyte solution containing ammonium bisulfate into the anode section of said electrolytic cell for use as the anolyte, said cathode and anode sections of said electrolytic cell being contained in a manner to prevent substantial amounts of persulfate values in said anolyte from mixing with said catholyte but permitting the free passage of hydrogen ions from said anolyte to said catholyte, passing an electric current through said catholyte and anolyte by means of a cathodic electrode contacting said catholyte and an anodic electrode contacting said anolyte, converting copper ions to copper at said cathodic electrode and forming ammonium bisulfate in said catholyte, converting sulfate ions to persulfate ions at said anode, recovering a second anolyte solution having an increased persulfate content, recovering a second catholyte solution containing ammonium bisulfate and having a decreased copper content for use in supplying sulfate values to anolyte solutions of succeeding regeneration cycles, and recycling said second anolyte solution to said ammonium persulfate etching solution for additional etching.

20. Process of claim 19 wherein said cooling is carried out at a temperature of from about 0 to 20° C.

21. Process of claim 19 wherein urea in amounts of from about 0.01% to 0.20% is added to said anolytes.

22. Process of claim 19 wherein ammonium thiocyanate in amounts of from about 0.01% to 0.20% is added to said anolytes.

23. Process of claim 19 wherein said electrolytic cell contains a diaphragm separating said anolyte and catholyte solutions.

#### References Cited

##### UNITED STATES PATENTS

|           |        |              |       |            |
|-----------|--------|--------------|-------|------------|
| 2,435,714 | 2/1948 | Fusco et al. | ----- | 204—237 XR |
| 2,589,982 | 3/1952 | Wood et al.  | ----- | 204—82     |
| 3,256,165 | 6/1966 | Williams     | ----- | 204—143    |

40 JOHN H. MACK, *Primary Examiner.*

D. R. JORDAN, *Assistant Examiner.*